

July 2, 1935.

W. A. WHITE ET AL

2,007,148

BUILDING CONSTRUCTION

Filed April 20, 1933



William A. White  
Edwin A. Kuhn  
INVENTORS

BY  
Frederick Griswold Jr.  
ATTORNEY

## UNITED STATES PATENT OFFICE

2,007,148

## BUILDING CONSTRUCTION

William A. White and Edwin A. Kunze, New York,  
N. Y.; Mary Mosetta White, executrix of the  
estate of said William A. White, deceased,  
assignor, by mesne assignments, to said Kunze

Application April 20, 1933, Serial No. 666,938

9 Claims. (Cl. 72—71)

This invention relates broadly to building construction and more particularly to masonry beams, girders, slabs, columns or the like, comprised in part of a reenforced cementitious composition. 5

One object of the present invention is to reduce the weight of such building construction without material sacrifice of strength, if any. To this end, a core is provided within the composite body, which is formed of any material lighter in weight than the cementitious composition, to wit, masonry, cement mortar or concrete that preferably surrounds the core on all sides and edges. Preferably such core comprises a fibrous material. 10

Another object of the invention is a core suitable for the purpose at hand. Accordingly, the core is preferably provided with a plurality of perforations extending therethrough, through which the cementitious composition extends and 15 bonds the material upon opposite faces of the core.

The invention also seeks a reenforced construction wherein the reenforcement opposes stresses in directions transverse to one another. Accordingly, reenforcing means extends between the spaced supports for the construction and other reenforcing means extends between and is supported by said first named reenforcing means. 20

A further object of the invention is a cementitious material for use in constructions according to the invention affording the maximum binding or bonding agency for the structural materials of larger bulk.

The invention also has to do with a construction which is practical from the standpoint of ease and cheapness of manufacture and durability and strength in use. In carrying the invention into effect, in its preferred embodiment, the composite construction comprises a pair of opposed, inwardly directed channels along opposite edges extending in the direction of the span and between which a reenforcing mesh sheet adjacent the lower face of the construction extends, the edges of the sheet being within the channels. A rectangular core of, say, fibrous material is disposed above the reenforcing mesh preferably terminating short of the adjacent margins of the channels, said core being formed with a plurality of vertically extending perforations. A hardened cementitious composition having high adhesive characteristics, entering the channels and extending therebetween, embeds and bonds the core and reenforcement and extends through the perforations in the core to bond the material on both sides thereof. 25

These and other objects of the invention and the means for their attainment will be more apparent from the following detailed description, taken in connection with the accompanying drawing illustrating a preferred embodiment by which the invention may be realized, and in which: 6

Figure 1 is a plan view showing the invention applied to a slab or beam construction, parts being broken away to disclose details; and

Figure 2 is a transverse sectional view taken on the plane indicated by the line 2—2 of Figure 1, looking in the direction of the arrows and showing particularly the manner in which those portions of the cementitious composition upon opposite sides of the core are bonded by material extending through perforations in the core. 10

The drawing illustrates a substantially square slab, embodying the invention, although it will be obvious that any desired relation between the length, width and depth of the slab, within limits, 20 may be availed of. Furthermore, the invention is equally applicable to other constructions, for instance, a beam, a column or other shapes comprising the use of cementitious materials and subjected to forces other than those involved in flexure. 25 Those ends or side edges of the slab or beam which extend between spaced supports 4, which the slab or beam spans, are defined by framing means preferably taking the form of inwardly facing channels 5, 6, the flanges of which are flush, respectively, with the upper and lower faces 1, 0 of the slab. Extending from one channel 5 to the other channel 6 is reenforcing means 11, 12. The reinforcement 11, 12 extends, practically, from edge to edge of those edges of the slab resting upon the spaced supports 4 thereby, with the channels 5, 6 taking up stresses in two directions at 90° to one another and thus taking advantage of the compressive resistance of the cementitious materials in both directions in contradistinction 35 to the compressive resistance of the cement in only one direction in a simple beam reinforced only in one direction. This reinforcement 11, 12, in the illustrated embodiment, extends into the channels 5, 6 and takes the form of a foraminous 40 sheet, such as the mesh or screen of spaced steel reenforcing rods 11 disposed in parallel relationship to each other adjacent to but slightly above the lower face 0 of the slab and similar spaced steel reenforcing rods 12 disposed also in parallel 45 relationship to each other and extending transversely of such first named rods 11 and preferably secured thereto, as by welding. As shown, there is a coating of cementitious substance over the 50 ends and surfaces of the rods. Obviously, other 55

forms of reenforcement, such as expanded metal, may be availed of in some situations.

A core 14 is disposed above the reenforcement. This core does not extend within the channels 5, 6 but, on the contrary, lies within the structure with its edges without the margins of the channels so that there is a material amount of cementitious composition 16 surrounding the core and between the core and channels and extending 10 within the channels. The core, as illustrated, is substantially rectangular and of material thickness and may or may not be in contact with the reenforcement 11, 12, depending upon the amount of cementitious material which finds its way therebetween. It is preferably formed of fibrous material, such as paper or wood pulp or the like, but any material which is lighter in weight than the masonry, cement mortar, concrete or other cementitious material that surrounds it on all sides, is 15 suitable.

At spaced points throughout its length and breadth, the core is perforated, as shown, with transversely extending perforations 18, that is, perforations, which, when the slab is in position, extend in a direction perpendicular to the longer faces of the slab. In manufacture, the channels are placed in position, the reenforcing sheet placed therebetween with the edges extending therein and, if desired, raised above the lower flanges of 30 the channels. A cementitious composition is then poured about the core and reenforcement and within the channels, as will be understood. Any cementitious composition having the desired characteristics, which can be poured in substantially 35 fluid state and which will harden or set upon standing, may be utilized. The composition flows all about the reenforcement and about the core and flows through the perforations 18 therein and extends within the channels 5, 6, so that the core 40 and reenforcement are wholly embedded therein and bonded thereto. In addition, the composition flows through the perforations 18 in the core and completely fills them and when the composition hardens, the material in the perforations serves 45 additionally as a bond between the material above and below the core 14. The cementitious material in the passages 18 assists in transferring the stresses from the compressive to the tensile side of the construction, as will be understood.

50 While any cementitious composition may be used it is preferred to use a cement having great capacity for adhesion to the core and reenforcing means. As an example, a plastic magnesia cement of the following formula has given satisfaction.

Parts by volume

|                   |    |
|-------------------|----|
| Calcined magnesia | 4  |
| Sand              | 5  |
| Talcum powder     | 1  |
| Silex             | 2½ |

To the foregoing is added a solution which shall preferably have the capacity to overcome or neutralize inherent defects in the magnesium oxide 65 of the mixture. Such a solution has taken the following form: Five parts by volume of a magnesium chloride solution of 22 Baumé and one part by volume of magnesium sulphate of 30 Baumé.

70 The talcum powder, of course, is added to lend a waterproofing characteristic to the cement.

The solution and graded aggregate are mixed to the proper consistency and the cement is ready for use.

75 A beam or slab construction manufactured in

the manner described has a strength substantially equal to that of the equivalent reinforced concrete construction without the core, but weighs considerably less. Steel is thus saved, in the construction, because of the reduced load. A slab has been tested which is about 51" square and 1¼" thick, and which has an effective span of 49". This slab was reenforced with electrically welded galvanized 10 gauge wire forming two inch square meshes, while the carrying channels taking the transverse reactions were bent from a three inch by one-eighth inch steel flat. The core was forty-eight inches square and three-quarters inches thick.

A total load of 421 pounds per square foot has been applied to this slab without ultimate failure thereof. This represents, in the given slab, a total load of 6738 pounds. With a total load of 3819 pounds, the maximum deflection at the center of the slab was .483 inches. In the safe working live load range, the deflections were as follows:

| Load                     | Deflection |
|--------------------------|------------|
| 50 lbs. per square foot  | 0.055"     |
| 75 lbs. per square foot  | 0.075"     |
| 100 lbs. per square foot | 0.092"     |
| 125 lbs. per square foot | 0.112"     |

It will thus be seen that building construction is provided by this invention which is considerably lighter in weight than that heretofore known although substantially the same strength is afforded, the lightness in weight being derived by virtue of the displacement of some of the material by material of a lighter weight, which lighter material adds nothing to the strength but which is so constructed as to permit the strength affording material to give to the construction the necessary strength.

A thin floor finish or flooring of an asphaltum mixture, for instance, even as thin as  $\frac{1}{16}$ ths of an inch, can be overlaid directly on slabs of this invention without cracking in use because of the adjacent channels of proximate slabs which support the load and distribute shear. This is because of the two-way reenforcement in the slab by which transverse reactions are taken up by the steel channels at the edges and which run in the direction of the span. It will be seen that because of the superior resistance to moving loads, that its reenforced edges will reduce the relative deflection at the joint to an appreciable extent which is of value in reducing the thickness of the flooring to be placed thereon, as it tends to inhibit cracking in floor finishes at the joints between the slabs.

Various modifications will occur to those skilled in the art in the composition, configuration and disposition of the component elements going to make up the invention as a whole, and no limitation is intended by the phraseology of the foregoing description or illustrations in the accompanying drawing.

What is claimed is:—

1. A composite structural member comprising in combination, framing means along opposite edges, reenforcing means disposed near one face of said structural member, a core of relatively light material adjacent the reenforcing means, said core being formed with a plurality of passages and a hardened adhesive cementitious composition extending between the framing means and in which the core and reenforcement are

embedded, said composition extending through the passages in the core and bonding the material on the sides thereof.

2. A composite structural member comprising, in combination, framing means along opposite edges, a reinforcing foraminous sheet disposed near one face of said structural member, a core of relatively light material adjacent the reinforcing sheet, said core being formed with a plurality of vertically extending perforations and a hardened cementitious composition extending between the framing means and in which the core and reinforcement are embedded, said composition extending through the perforations in the core and bonding the material on both sides thereof.

3. A composite structural member comprising, in combination, framing means along opposite edges, reenforcing means disposed near one face of said structural member and extending from edge to edge transversely of said framing means and interconnecting therewith a load bearing core of relatively light material adjacent the reenforcing means and a hardened adhesive cementitious composition having the characteristics of a plastic cement comprising magnesia, sand and a filler extending between the framing means and in which the core and reenforcement are embedded, said composition being bonded to the core and reenforcing means.

4. A composite structural member comprising, in combination, framing means along opposite edges, reenforcing means disposed near one face of said structural member and in overlapping relationship with said framing means, a foraminous core of relatively light material adjacent the reenforcing means in non-overlapping relationship with the framing means and a hardened cementitious composition interlocked with the framing means and in which the core and reenforcing means are embedded, said composition extending through the perforations in the core and bonding the material on both sides thereof.

5. A composite structural member comprising, in combination, a pair of opposed, inwardly directed channels along opposite edges, a reenforcing mesh sheet disposed near one face of the structural member and extending within the channels, a core of relatively light material adjacent the reenforcing mesh and terminating without the margins of the channels, said core being formed with a plurality of vertically extending perforations and a hardened cementitious composition extending between the channels and in which the core and reenforcement are embedded, said composition extending through the perforations in the core and bonding the material on both sides thereof.

6. A composite structural member comprising, in combination, a pair of opposed, inwardly directed channels along opposite edges, a reenforcing mesh sheet disposed near one face of the structural member and extending within the channels, a rectangular core of fibrous material disposed above the reenforcing mesh and terminating without the margins of the channels, said core being formed with a plurality of vertically extending perforations and a hardened cementitious composition extending between the channels and in which the core and reinforcement are embedded, said composition extending through the perforations in the core and bonding the material on both sides thereof.

7. A composite structural member comprising, in combination, a pair of opposed, inwardly directed channels along opposite edges, a reenforcing mesh sheet near the lower face of the structural member and comprising steel reenforcing rods disposed in parallel relationship and spaced steel reenforcing rods disposed in parallel relationship and extending transversely of said first named rods and secured thereto, the ends of said rods extending within the channels, a rectangular core of fibrous material disposed above the reenforcing mesh whereof the edges are disposed outwardly of the margins of the channels, said core being formed with a plurality of vertically extending perforations and a hardened cementitious composition entering the channels and extending therebetween and in which the core and reenforcement are embedded, said composition extending through the perforations in the core and bonding the material on both sides thereof.

8. A composite structural member comprising, in combination, framing means along opposite edges, reenforcing means disposed near one face of said structural member and in overlapping relationship with said framing means, a foraminous load bearing core of relatively light material adjacent the reenforcing means in non-overlapping relationship with the framing means, and a hardened cementitious composition interlocked with the framing means and in which the core and reenforcing means are embedded and adhered, said composition comprising a plastic magnesia cement.

9. A composite structural member, comprising, in combination, reenforcing means disposed near a face of said structural member, a load bearing core of relatively light material adjacent the reenforcing means and a hardened adhesive cementitious composition in which the core and reenforcement is embedded, said composition being bonded to the core and reenforcing means.

WILLIAM A. WHITE.

EDWIN A. KUNZE.